

## UNITED STATES PATENT OFFICE.

ROBERT ILLEMANN, OF GLASGOW, SCOTLAND.

## SOLID OIL FUEL.

No Drawing.

Application filed July 31, 1922. Serial No. 578,804.

*To all whom it may concern:*

Be it known that I, ROBERT ILLEMANN, of 54 Scott Street, Port Dundas, Glasgow, Scotland, a citizen of the United States of 5 America, have invented a certain new and useful Solid Oil Fuel, of which the following is a specification.

The object of this invention is the production of solid oil fuel from oil and wet peat, 10 By the term "oil" I not only desire to include mineral, animal, vegetable, or fish oil, but also greases, waxes, oil residues, and other oleaginous or bituminous substances which are normally in a solid or semisolid 15 condition and can be converted into liquid oils by the application of a solvent or otherwise.

At present it is common practice to employ liquid fuel, usually heavy oils, such as 20 creosote, Texan or Mexican oils, for the purpose of firing the steam boilers of ships and of industrial works, heating metallurgical and other furnaces, etc., although not for domestic purposes, it being usual to spray 25 the oil in a finely atomized condition by means of burners or sprayers. In all cases burners and special plant have to be installed which are more or less costly and are only useful for their specific purpose. My 30 invention obviates the use of such burners and plant and at the same time renders it unnecessary to employ oil tanks, barrels, or vessels in which, at present, the oil must be kept or carried.

35 My invention aims at supplying the oil fuel in a solid condition and preferably in the form of briquettes, nuggets, blocks, lumps, or the like, so that it can be handled and used as readily as coal or wood.

40 I have found that when I take peat which may be more or less fibrous (preferably the black variety) containing a large percentage of water—if the peat does not contain sufficient I may increase the quantity of water— 45 and place it in a vessel and subject it to an operation, such as grinding and agitation, so as to break up the fibrous matters therein and reduce the peat to a moist coagulate or thickened curd-like condition and then add, 50 during the operation, a quantity of mineral or other oil in a liquid condition, that the oil, peat and water becomes a homogeneous mass which gradually, under continued agitation, assumes the consistency of a stiff 55 paste. As the peat contains bituminous

matters naturally these will amalgamate with the oil. The substance thus produced can be formed, pressed, or moulded, into any desired shape such as briquettes, lumps, blocks, or slabs.

60 When it is desired to form the substance into briquettes or blocks a machine, of the brick-making type, can be used for pressing the plastic substance through a cylinder having either an oval or square mouthpiece, 65 the extruded substance being cut by a wire or knife into blocks or pieces of the desired size. The blocks can then be stacked for drying, either by the action of air or by artificial heat. If so desired, in order to expedite the drying, we may heat the whole mass during the agitating and grinding operation and before moulding.

70 During the drying process a very peculiar action takes place, as, after the water has evaporated, it will be found the oil has been left behind, it being absorbed in the microscopic cells of the peat formerly occupied by the water. As the block dries, it 75 solidifies into a dry solid tough briquette 80 which can be handled, packed, or stacked with perfect safety without the oil separating or exuding from the briquette. When the block is cut by a knife it shows a clean 85 smooth surface.

When placed in a furnace or in domestic stoves and ranges the oily matters in the 90 briquettes burn freely and a complete combustion thereof takes place with only one to three per cent, or so, of ash. The briquette 90 burns with a bright hot flame somewhat similar to oil when used in a spray burner.

For example, I have found, in practice, 95 that 16 oz. (avoird.) good black wet peat treated as aforesaid to bring it to a coagulated condition in combination with 4 oz. crude mineral oil will produce a briquette which, after the water has been evaporated therefrom, measures about 11½ cubic inches and weighs about 7 oz. and it will be found 100 to contain 3 oz. of peat (dry) and 4 oz. of oil so that the small bulk of peat contains or carries a greater bulk of oil. The block constitutes an oil briquette in which the oil is combined with the peat molecules and it 105 appears dry and solid and the oil does not exude or separate therefrom.

The amount of oil used for making the fuel can be varied and regulated according to the calorific value desired, per cubic inch,

of the briquette and according to the amount of bituminous or oily matter originally present in the peat.

Having now fully described my invention 5 what I claim and desire to secure by Letters Patent is:—

1. The method of manufacturing solid oil fuel from oil and peat which consists in providing a quantity of peat which contains 10 an excess quantity of water and grinding and thoroughly breaking up the peat and agitating the peat and water until it assumes a coagulated condition, then adding oil and mixing the mixture until the whole becomes 15 a homogeneous mass of a thick plastic consistency and then moulding the same into blocks, briquettes and the like, the resulting mass having incorporated therein oil in excess of the peat.
2. The method of manufacturing solid oil fuel from oil and peat which consists in pro- 20

viding peat containing an excess quantity of water and grinding and thoroughly breaking up the peat so as to freely expose the cellular structure of the peat and so that a 25 portion of the oil will not only be absorbed by the peat but the peat will also serve as a binding agent and carrier for excess oil, then mixing the peat and water until it assumes a coagulated condition, then adding 30 an excess quantity of oil and mixing it until the whole becomes a homogeneous mass of a plastic consistency, and then moulding the same, the resulting product having incorporated therein oil in excess of the peat. 35

In testimony whereof I affix my signature in presence of two witnesses.

ROBERT ILLEMANN.

Witnesses:

MARY GREEN,  
AGNES GILMOUR.